

# United States Patent Office

2,698,837

Patented Jan. 4, 1955

1

2,698,837

## FUNCTIONAL FLUIDS

Harry R. Gamrath and Roger E. Hatton, St. Louis, Mo., assignors to Monsanto Chemical Company, St. Louis, Mo., a corporation of Delaware

No Drawing. Application November 15, 1950,  
Serial No. 195,913

8 Claims. (Cl. 252—78)

This invention relates to functional fluids; more specifically, this invention relates to improved functional fluid compositions comprising a mixture of dialkyl monoaryl phosphate esters having the formula



wherein  $\text{R}_1$  and  $\text{R}_2$  represent alkyl radicals, preferably containing from 1 to 18 carbon atoms, and  $\text{R}_3$  represents an aryl radical, and dialkyl esters of aliphatic dicarboxylic acids having the formula



wherein  $\text{R}_4$  and  $\text{R}_5$  represent alkyl radicals containing from 4 to 10 carbon atoms and  $n$  is an integer from 2 to 8 inclusive.

Many different types of materials are utilized as functional fluids and functional fluids are used in many different types of applications. Such fluids have been used as synthetic lubricants, damping fluids, bases for greases, force transmission fluids (hydraulic fluids) and as filter mediums for air conditioning systems. Because of the wide variety of application and the varied conditions under which functional fluids are utilized, the properties desired in a good functional fluid necessarily vary with the particular application in which it is to be utilized with each individual application calling for a functional fluid having a specific class of properties. Of primary importance in a functional fluid is its viscosity characteristic over a wide temperature range and blends of different types of functional fluids are often resorted to in order to obtain a particular functional fluid having a particular viscosity characteristic. Knowing the viscosity characteristics of two separate functional fluids, it has heretofore been possible in the case of certain materials to determine the ratio in which these two fluids must be combined in order to obtain a new fluid having viscosity characteristics intermediate or resulting from the two individual functional fluids. ASTM Method D341-43, Appendix, has afforded a convenient method in certain instances of determining or predicting the viscosity characteristics of a mixture composed of two functional fluids whose viscosity characteristics individually are known.

Various esters of ortho-phosphoric acid and of aliphatic dicarboxylic acids have been found to have utility as functional fluids. Among the ortho-phosphate esters, we have found that the dialkyl monoaryl phosphates as a class possess exceptional properties in functional fluids. Such dialkyl monoaryl phosphates are superior to the trialkyl phosphates because they are generally less volatile. The dialkyl monoaryl phosphate esters are superior to the triaryl phosphates and the monoalkyl diaryl phosphates because they possess improved viscosity characteristics at low temperatures. It has been found that the dialkyl monoaryl phosphate esters may be utilized individually as functional fluids or mixtures of the dialkyl monoaryl phosphate esters may be utilized to obtain functional fluids having particular viscosity characteristics unattainable by the phosphate esters individually, but obtainable through mixtures of the phosphate esters. When utilized as mixtures, the mixtures have been found to behave as would be expected or predicted. In other words, the actual viscosity of a mixture of these dialkyl monoaryl phosphate esters is essentially the same as the

2

predicted viscosity of the mixture when determined in accordance with ASTM Method D341-43. In like fashion, the alkyl esters of aliphatic dicarboxylic acids are utilized individually in certain applications as functional fluids, while in others, mixtures of the alkyl esters of aliphatic dicarboxylic acids are utilized in order to obtain a particular viscosity characteristic. As in the case of mixtures of the dialkyl monoaryl phosphate esters, mixtures of the esters of aliphatic dicarboxylic acids have been found to behave as would be expected in that the actual viscosity of such mixtures is essentially the same as the predicted viscosity when determined in accordance with ASTM Method D341-43. The viscosity characteristics of such compositions are illustrated in the following 15 Table A:

TABLE A

| 20 | Composition                                       | Viscosity in Centistokes at -40° F. |           |
|----|---------------------------------------------------|-------------------------------------|-----------|
|    |                                                   | Observed                            | Predicted |
| 25 | Di- <i>n</i> -butyl succinate                     | *18.9                               |           |
|    | Diamyl adipate                                    | 192                                 |           |
|    | Di(6-methylheptyl) adipate                        | 1,270                               |           |
|    | Di(2-ethylhexyl) sebacate                         | 1,600                               |           |
|    | 2-Ethylhexyl <i>n</i> -butyl phenyl phosphate     | 641                                 |           |
|    | 2-Ethylhexyl capryl phenyl phosphate              | 1,710                               |           |
|    | Di(2-ethylhexyl) phenyl phosphate                 | 1,820                               |           |
|    |                                                   | *161                                |           |
| 30 | 2-Ethylhexyl <i>n</i> -butyl cresyl phosphate     | 1,370                               |           |
|    | 2-Ethylhexyl sec-butyl cresyl phosphate           | 3,500                               |           |
|    | 2-Ethylhexyl 2-butyloctyl cresyl phosphate        | 6,200                               |           |
|    | 50% Diethyl adipate                               | 503                                 | 510       |
|    | 50% Di(6-methylheptyl) sebacate                   |                                     |           |
|    | 50% Diethyl adipate                               | 512                                 | 495       |
| 35 | 50% 2-Ethylhexyl <i>n</i> -butyl phenyl phosphate | 1,090                               | 1,100     |
|    | 50% Di(2-ethylhexyl) phenyl phosphate             |                                     |           |
|    | 50% 2-Ethylhexyl <i>n</i> -butyl cresyl phosphate | 2,850                               | 2,800     |
|    | 50% 2-Ethylhexyl 2-butyloctyl cresyl phosphate    |                                     |           |

\* Viscosity at 0° F.

40 While the alkyl esters of aliphatic dicarboxylic acids have some utility per se, as functional fluids, particularly as a result of their exceptionally low viscosities at low temperatures, their relatively poor flammability characteristics restricts their utility to certain specialty applications. The dialkyl monoaryl phosphates on the other hand find much wider utility because of their excellent fire-retardancy and relatively low viscosity at low temperatures. However, notwithstanding the favorable 45 properties exhibited by the dialkyl monoaryl phosphate esters, certain functional fluid applications require a relatively non-flammable functional fluid having even a lower viscosity at low temperatures than do the dialkyl monoaryl phosphate esters per se.

50 It is an object of this invention to provide new and improved compositions having utility as functional fluids. It is a further object of this invention to provide new and improved compositions having increased utility as functional fluids at low temperatures. A still further object of this invention is to provide an improved method 55 of transmitting power in and lubricating the frictional parts of a hydraulic system having a pump therein supplying the power. Another object of this invention is to provide a hydraulic system having improved performance 60 characteristics. Further objects will become apparent from a description of this invention.

65 It has now been discovered that mixtures of the dialkyl monoaryl phosphate esters hereinbefore described and the dialkyl esters of aliphatic dicarboxylic acids hereinbefore described behave abnormally in that the viscosity of such mixtures does not correspond to the predicted value, but is actually much lower, resulting in functional fluids having unexpected, unpredictable and surprisingly enhanced physical properties. According to one embodiment of this invention, therefore, improved functional 70 fluids, characterized by exceptionally low viscosity characteristics at low temperatures and excellent fire-retardancy, comprising a mixture of the dialkyl monoaryl phosphate esters hereinbefore described and the dialkyl esters of aliphatic dicarboxylic acids hereinbefore described are provided. The following examples are illustrative, but

not limitative, of the novel improved functional fluids of this invention:

*Example I*

An improved functional fluid was prepared by mixing 10 parts by weight of diamyl adipate and 90 parts by weight of di(2-ethylhexyl) phenyl phosphate. The resultant functional fluid had the following properties:

|                                |               |
|--------------------------------|---------------|
| Specific gravity at 25°/25° C. | 0.9875.       |
| N <sub>D</sub> <sup>25</sup>   | 1.4659.       |
| Pour point                     | Below -70° F. |
| Viscosity, centistokes:        |               |
| At 210° F.                     | 2.21.         |
| At 100° F.                     | 8.02.         |
| At -40° F.                     | 1340.         |
| Predicted viscosity at -40° F. | 1450.         |

*Example II*

An improved functional fluid was prepared by mixing 10 parts by weight of di-isoamyl adipate and 90 parts by weight of 2-ethylhexyl n-butyl phenyl phosphate. The resultant functional fluid had the following properties:

|                                |               |
|--------------------------------|---------------|
| Specific gravity at 25°/25° C. | 1.0129.       |
| N <sub>D</sub> <sup>25</sup>   | 1.4663.       |
| Pour point                     | Below -70° F. |
| Viscosity, centistokes:        |               |
| At 210° F.                     | 1.82.         |
| At 100° F.                     | 5.93.         |

*Example III*

An improved functional fluid was prepared by mixing 10 parts by weight of di(6-methylheptyl) adipate and 90 parts by weight of 2-ethylhexyl sec-butyl p-chlorophenyl phosphate. The resultant functional fluid had the following properties:

|                                |               |
|--------------------------------|---------------|
| Specific gravity at 25°/25° C. | 1.0756.       |
| N <sub>D</sub> <sup>25</sup>   | 1.4800.       |
| Pour point                     | Below -70° F. |
| Viscosity, centistokes:        |               |
| At 210° F.                     | 2.53.         |
| At 100° F.                     | 11.07.        |

*Example IV*

An improved functional fluid was prepared by mixing 25 parts by weight of diamyl adipate and 75 parts by weight of 2-ethylhexyl capryl phenyl phosphate. The resultant functional fluid had the following properties:

|                                |               |
|--------------------------------|---------------|
| Specific gravity at 25°/25° C. | 0.9776.       |
| N <sub>D</sub> <sup>25</sup>   | 1.4600.       |
| Pour point                     | Below -70° F. |
| Viscosity, centistokes:        |               |
| At 210° F.                     | 2.10.         |
| At 100° F.                     | 7.33.         |
| At -40° F.                     | 857.          |
| Predicted viscosity at -40° F. | 1000.         |

*Example V*

An improved functional fluid was prepared by mixing 25 parts by weight of di(2-ethylbutyl) adipate and 75 parts by weight of n-octyl n-butyl phenyl phosphate. The resultant functional fluid had the following properties:

|                                |               |
|--------------------------------|---------------|
| Specific gravity at 25°/25° C. | 0.9955.       |
| N <sub>D</sub> <sup>25</sup>   | 1.4605.       |
| Pour point                     | Below -70° F. |
| Viscosity, centistokes:        |               |
| At 210° F.                     | 1.92.         |
| At 100° F.                     | 6.03.         |

*Example VI*

An improved functional fluid was prepared by mixing 50 parts by weight of di-isoamyl adipate and 50 parts by weight of 2-ethylhexyl n-butyl phenyl phosphate. The resultant functional fluid had the following properties:

|                                |               |
|--------------------------------|---------------|
| Specific gravity at 25°/25° C. | 0.9809.       |
| N <sub>D</sub> <sup>25</sup>   | 1.4518.       |
| Pour point                     | Below -70° F. |
| Viscosity, centistokes:        |               |
| At 210° F.                     | 1.73.         |
| At 100° F.                     | 5.29.         |
| At 0° F.                       | 49.7.         |
| At -40° F.                     | 327.          |
| Predicted viscosity at -40° F. | 370.          |

*Example VII*

An improved functional fluid was prepared by mixing 50 parts by weight of diamyl adipate and 50 parts by weight of 2-ethylhexyl sec-butyl cresyl phosphate. The resultant functional fluid had the following properties:

|                                |               |
|--------------------------------|---------------|
| Specific gravity at 25°/25° C. | 0.9780.       |
| N <sub>D</sub> <sup>25</sup>   | 1.4541.       |
| Pour point                     | Below -70° F. |
| Viscosity, centistokes:        |               |
| At 210° F.                     | 2.07.         |
| At 100° F.                     | 6.68.         |
| At -40° F.                     | 537.          |
| Predicted viscosity at -40° F. | 750.          |

*Example VIII*

An improved functional fluid was prepared by mixing 50 parts by weight of di(2-ethylbutyl) adipate and 50 parts by weight of 2-ethylhexyl isobutyl phenyl phosphate. The resultant functional fluid had the following properties:

|                                |               |
|--------------------------------|---------------|
| Specific gravity at 25°/25° C. | 0.9828.       |
| N <sub>D</sub> <sup>25</sup>   | 1.4560.       |
| Pour point                     | Below -70° F. |
| Viscosity, centistokes:        |               |
| At 210° F.                     | 2.74.         |
| At 100° F.                     | 6.19.         |
| At -40° F.                     | 525.          |
| Predicted viscosity at -40° F. | 640.          |

*Example IX*

An improved functional fluid was prepared by mixing 50 parts by weight of di(2-ethylbutyl) adipate and 50 parts by weight of n-butyl sec-tetradecyl phenyl phosphate. The resultant functional fluid had the following properties:

|                                |               |
|--------------------------------|---------------|
| Specific gravity at 25°/25° C. | 0.9374.       |
| N <sub>D</sub> <sup>25</sup>   | 1.4500.       |
| Pour point                     | Below -70° F. |
| Viscosity, centistokes:        |               |
| At 210° F.                     | 2.24.         |
| At 100° F.                     | 8.05.         |
| At -40° F.                     | 1006.         |
| Predicted viscosity at -40° F. | 1300.         |

*Example X*

An improved functional fluid was prepared by mixing 50 parts by weight of di(6-methylheptyl) adipate and 50 parts by weight of 2-ethylhexyl capryl phenyl phosphate. The resultant functional fluid had the following properties:

|                                |               |
|--------------------------------|---------------|
| Specific gravity at 25°/25° C. | 0.9565.       |
| N <sub>D</sub> <sup>25</sup>   | 1.4570.       |
| Pour point                     | Below -70° F. |
| Viscosity, centistokes:        |               |
| At 210° F.                     | 2.53.         |
| At 100° F.                     | 9.21.         |
| At -40° F.                     | 1360.         |
| Predicted viscosity at -40° F. | 1475.         |

*Example XI*

An improved functional fluid was prepared by mixing 50 parts by weight of di-n-butyl adipate and 50 parts by weight of di(2-ethylhexyl) phenyl phosphate. The resultant functional fluid had the following properties:

|                                |        |
|--------------------------------|--------|
| Specific gravity at 25°/25° C. | 0.9735 |
| N <sub>D</sub> <sup>25</sup>   | 1.4496 |
| Viscosity, centistokes:        |        |
| At 210° F.                     | 1.60   |
| At 100° F.                     | 5.01   |
| At -40° F.                     | 480    |
| At 0° F.                       | 42.5   |
| Predicted viscosity at 0° F.   | 57.0   |

The predicted and observed viscosities of this composition were compared at 0° F. since di-n-butyl adipate crystallizes at about -9° F.

*Example XII*

An improved functional fluid was prepared by mixing 50 parts by weight of di(2-ethylhexyl) sebacate and 50 parts by weight of 2-ethylhexyl n-butyl phenyl phos-

phate. The resultant functional fluid had the following properties:

|                                |               |
|--------------------------------|---------------|
| Specific gravity at 25°/25° C. | 0.9648.       |
| N <sub>D</sub> <sup>25</sup>   | 1.4587.       |
| Pour point                     | Below -70° F. |
| Viscosity, centistokes:        |               |
| At 210° F.                     | 2.49.         |
| At 100° F.                     | 8.87.         |

*Example XIII*

An improved functional fluid was prepared by mixing 50 parts by weight of di(2-ethylhexyl) sebacate and 50 parts by weight of 2-ethylhexyl 2-butyloctyl cresyl phosphate. The resultant functional fluid had the following properties:

|                                |               |
|--------------------------------|---------------|
| Specific gravity at 25°/25° C. | 0.9362.       |
| N <sub>D</sub> <sup>25</sup>   | 1.4588.       |
| Pour point                     | Below -70° F. |
| Viscosity, centistokes:        |               |
| At 210° F.                     | 3.57.         |
| At 100° F.                     | 13.69.        |
| At -40° F.                     | 2840.         |
| Predicted viscosity at -40° F. | 3150.         |

*Example XIV*

An improved functional fluid was prepared by mixing 50 parts by weight of di-n-butyl succinate and 50 parts by weight of di(2-ethylhexyl) phenyl phosphate. The resultant functional fluid had the following properties:

|                                |        |
|--------------------------------|--------|
| Specific gravity at 25°/25° C. | 0.9833 |
| N <sub>D</sub> <sup>25</sup>   | 1.4481 |
| Viscosity, centistokes:        |        |
| At 210° F.                     | 1.68   |
| At 100° F.                     | 4.98   |
| At -40° F.                     | 284    |
| At 0° F.                       | 43.6   |
| Predicted viscosity at 0° F.   | 50.5   |

The predicted and observed viscosities of this composition were compared at 0° F. since di-n-butyl succinate crystallizes at about -19° F.

In addition to the dialkyl monoaryl phosphate esters utilized in the preceding examples, the following ortho-phosphate esters are further examples of dialkyl monoaryl phosphate esters which may be utilized to prepare improved functional fluids in accordance with this invention:

| DIALKYL MONOARYL ORTHO-PHOSPHATE ESTERS           |  |
|---------------------------------------------------|--|
| Amyl isoamyl phenyl phosphate                     |  |
| Diamyl phenyl phosphate                           |  |
| 2-ethylhexyl methyl phenyl phosphate              |  |
| 2-ethylhexyl propyl phenyl phosphate              |  |
| 2-ethylhexyl sec-butyl phenyl phosphate           |  |
| 2-ethylhexyl n-butyl cresyl phosphate             |  |
| Dicapryl phenyl phosphate                         |  |
| Nonyl n-hexyl o-chlorophenyl phosphate            |  |
| Dodecyl decyl phenyl phosphate                    |  |
| n-Hexadecyl isopropyl phenyl phosphate            |  |
| Butoxyethyl 3,5,5-trimethylhexyl cresyl phosphate |  |
| Butoxyethyl n-octyl o-methoxyphenyl phosphate     |  |

While those dialkyl monoaryl phosphate esters wherein the alkyl substituents are unsubstituted constitute a preferred embodiment of this invention, the alkyl substituents may be substituted with one or more unreactive substituents. Thus, the alkyl groups of the hereinbefore described phosphate esters may be substituted with nitro groups, aryl groups such as phenyl, alkoxy groups such as ethoxy, butoxy, isopropoxy, etc. In like manner, those dialkyl monoaryl phosphate esters wherein the aryl group is a phenyl group, which may be substituted or unsubstituted, constitutes a preferred embodiment of this invention. Typical of such aryl groups are the phenyl, cresyl, higher alkyl substituted phenyl, alkoxy substituted phenyl, halogen substituted phenyl and nitro substituted phenyl groups.

The novel functional fluids of this invention may be prepared by merely mixing the dialkyl monoaryl phosphate esters hereinbefore described and the dialkyl esters of aliphatic dicarboxylic acids in any desired proportion, dependent upon the resultant physical properties desired. A particularly preferred class of functional fluids exhibiting significantly enhanced physical properties are those containing the hereinbefore described dialkyl monoaryl

phosphate esters and from about .5 to about 75% by weight of total composition of a dialkyl ester of an aliphatic dicarboxylic acid.

The novel functional fluids of this invention comprising a mixture of the hereinbefore described dialkyl monoaryl phosphate esters and dialkyl esters of aliphatic dicarboxylic acids may be used per se as functional fluids or they may be used in combination with oxidation inhibitors, rust inhibitors, anti-foaming agents, detergents, viscosity index improvers compatible therewith, etc., whenever specific uses require such addition agents. Particularly useful functional fluids are those compositions comprising a mixture of a hereinbefore described dialkyl monoaryl phosphate ester, a dialkyl ester of an aliphatic dicarboxylic acid and a minor amount, such as from about 0.2 to about 10% by weight of total composition of a viscosity index improver, such as a polymerized alkyl methacrylate (preferably the poly octyl methacrylate) or an alkylated polymerized styrene, such as polymerized styrene of a molecular weight within the range of 10,000 to 150,000 which has been alkylated with olefins containing from 6 to 15 carbon atoms.

As a result of the excellent physical properties of the functional fluids particularly described in the preceding examples, improved hydraulic pressure devices can be prepared in accordance with this invention which comprise in combination a fluid chamber and an actuating fluid in said chamber, said fluid comprising a mixture of a dialkyl monoaryl phosphate ester as hereinbefore described and a dialkyl ester of an aliphatic dicarboxylic acid as hereinbefore described. In such a hydraulic apparatus wherein a movable member is actuated by the above described functional fluid, performance characteristics are obtainable which are superior to those heretofore obtainable.

Because of the excellent flammability characteristics of the functional fluids of this invention, their exceptionally low pour points, and high inherent lubricity, the functional fluids of this invention may be utilized in those hydraulic systems wherein power must be transmitted and the frictional parts of the system lubricated by the hydraulic fluid utilized. Thus, the novel functional fluids of this invention find exceptional utility in the transmission of power in a hydraulic system having a pump therein supplying the power for the system. In such a system, the parts which are so lubricated include the frictional surfaces of the source of power, namely the pump, valves, operating pistons and cylinders, fluid motors, and in some cases, for machine tools, the ways, tables and slides. The hydraulic system may be of either the constant-volume or the variable-volume type of system.

The pumps may be of various types, including the piston-type pump, more particularly the variable-stroke piston pump, the variable-discharge or variable displacement piston pump, radial-piston pump, axial-piston pump, in which a pivoted cylinder block is adjusted at various angles with the piston assembly, for example, the Vickers Axial-Piston Pump, or in which the mechanism which drives the pistons is set at an angle adjustable with the cylinder block; gear-type pump, which may be spur, helical or herringbone gears, variations of internal gears, or a screw pump; or vane pumps. The valves may be stop valves, reversing valves, pilot valves, throttling valves, sequence valves or relief valves. Fluid motors are usually constant- or variable-discharge piston pumps caused to rotate by the pressure of the hydraulic fluid of the system with the power supplied by the pump power source. Such a hydraulic motor may be used in connection with a variable-discharge pump to form a variable-speed transmission.

What is claimed is:

1. A functional fluid comprising essentially a mixture of 25 to 90 parts by weight of dialkyl monoaryl phosphate ester having the formula

75



80  
wherein R<sub>1</sub> and R<sub>2</sub> each represents an alkyl radical containing from 1 to 18 carbon atoms, and R<sub>3</sub> represents an aryl radical, and 10 to 75 parts by weight of dialkyl ester

of an aliphatic dicarboxylic acid having the formula  
 $R_4OOC(CH_2)_nCOOR_5$

wherein  $R_4$  and  $R_5$  each represents an alkyl radical containing from 4 to 10 carbon atoms, and  $n$  is an integer from 2 to 8 inclusive.

2. A functional fluid comprising essentially a mixture of 50 to 90 parts by weight of dialkyl monoaryl phosphate ester having the formula



wherein  $R_1$  and  $R_2$  each represents an alkyl radical containing from 4 to 14 carbon atoms, and  $R_3$  represents a phenyl radical, and 10 to 50 parts by weight of dialkyl ester of an aliphatic dicarboxylic acid having the formula



wherein  $R_4$  and  $R_5$  each represents an alkyl radical containing from 4 to 10 carbon atoms, and  $n$  is an integer from 2 to 8 inclusive.

3. A functional fluid comprising essentially a mixture of 50 to 90 parts by weight of octyl butyl phenyl phosphate and 10 to 50 parts by weight of dialkyl ester of an aliphatic dicarboxylic acid having the formula



wherein  $R_4$  and  $R_5$  each represents an alkyl radical containing from 4 to 10 carbon atoms, and  $n$  is an integer from 2 to 8 inclusive.

4. A functional fluid comprising essentially a mixture of 50 to 90 parts by weight of 2-ethylhexyl n-butyl phenyl phosphate and 10 to 50 parts by weight of di-isoamyl adipate.

5. A functional fluid comprising essentially a mixture of 50 to 90 parts by weight of n-octyl n-butyl phenyl phosphate and 10 to 50 parts by weight of di(2-ethylbutyl) adipate.

6. A functional fluid comprising essentially a mixture of 50 to 90 parts by weight of 2-ethylhexyl sec-butyl cresyl phosphate and 10 to 50 parts by weight of diamyl adipate.

7. A functional fluid comprising essentially a mixture of 50 to 90 parts by weight of 2-ethylhexyl capryl phenyl phosphate and 10 to 50 parts by weight of di(6-methylheptyl) adipate.

8. A functional fluid comprising essentially a mixture of 50 to 90 parts by weight of 2-ethylhexyl n-butyl phenyl phosphate and 10 to 50 parts by weight of di(2-ethylhexyl) sebacate.

20

References Cited in the file of this patent

UNITED STATES PATENTS

|           |                  |               |
|-----------|------------------|---------------|
| 2,342,414 | Magill           | Feb. 22, 1944 |
| 2,481,372 | Von Fuchs et al. | Sept. 6, 1949 |
| 2,512,582 | Pluedeman        | June 20, 1950 |
| 2,542,785 | Walker           | Feb. 20, 1951 |

FOREIGN PATENTS

|    |         |               |               |
|----|---------|---------------|---------------|
| 30 | 457,548 | Great Britain | Aug. 24, 1935 |
|    | 524,937 | Great Britain | Aug. 19, 1940 |